# EUROPEAN PATENT SPECIFICATION

(11) **EP 0 960 235 B1**
(45) Date of publication and mention of the grant of the patent: **24.04.2002**
(21) Application number: 98900506.1
(22) Date of filing: 19.01.1998
(51) Int. Cl.: D21C 9/147, D21C 9/10

(54) **OXYGEN DELIGNIFICATION PROCESS OF PULP**
DELIGNIFIZIERUNG VON ZELLSTOFF MIT SAUERSTOFF
PROCEDE DE DELIGNIFICATION A L'OXYGENE DE PATE A PAPIER

(30) Priority: 21.01.1997 US 786216
(43) Date of publication of application: 01.12.1999
(73) Proprietor: UNIVERSITY OF NEW BRUNSWICK, Fredericton, New Brunswick E3B 5A3 (CA)
(72) Inventor: NI, Yonghao, Fredericton, New Brunswick E3C 1M1 (CA); VAN HEININGEN, Adriaan, R., P., Mouth of Keswick, New Brunswick E0H 1N0 (CA); KANG, Guo, Jun, Fredericton, New Brunswick E3B 2T5 (CA); SKOTHOS, Anastasios, Montreal, Quebec H1Z 3H8 (CA)
(74) Representative: Schwarzensteiner, Marie-Luise
(86) International application number: CA9800020
(87) International publication number: WO9831872

(56) References cited:
- WO-A-96/05364
- CA-A- 2 157 154
- DE-A- 3 809 332
- FR-A- 2 692 917
- NI, Y. ET AL: "An improved oxygen delignification for magnesium based sulfite process." 1997 PULPING CONFERENCE-TAPPI PROCEEDINGS. TAPPI PRESS, 19 October 1997, pages 551-557, XP002065280

## Description

### FIELD OF THE INVENTION

The present invention is concerned with a single stage process for decreasing carbohydrate degradation of sulphite pulps during the O_{MgO} process by the addition of a catalytic amount of sodium borohydride *in situ* to provide a pulp with enhanced strength properties and increased viscosity.

### BACKGROUND OF THE INVENTION

Because of increasing environmental concerns worldwide, pulp and paper mills discharge effluents are constantly under scrutiny to ensure that environmental regulations are followed. Because of the high costs involved in the treatment of effluents before their release in the environment, a great deal of research is directed to the modification of current pulp and paper production processes. The research concentrates its efforts in replacing toxic reagents with more environmentally friendly products. A further benefit sought with such changes is that effluents will hopefully require fewer costly conditioning treatments before their release in the environment.

In the various processes proposed in the literature, the oxygen delignification technology is one of the available options towards this direction. Conventionally, oxygen delignification technology uses sodium hydroxide as the alkaline source and the resulting effluent produced can therefore he incorporated into the chemical recovery system of the process for preparing kraft pulps because the same reagent, namely sodium hydroxide, is used, and therefore, there is no reagent interference. On the other hand, the effluent from the sodium hydroxide-based oxygen delignification process (referred to as the O_{NaOH} technology herein) cannot be sent to the recovery system of the magnesium-based sulphite process because, obviously, the sodium salts are not compatible with the magnesium-based sulphite recovery process. Several publications have therefore concluded that magnesium oxide-based oxygen delignification technology, referred to as O_{MgO} herein, is preferred for magnesium-based sulphite pulping processes. (see for example Bokstrom et al., *Pulp and Paper Canada*, 1992, 92 (11), 38; and Luo et al., *Tappi Journal*, 1992, 75 (6), 183).

Sodium hydroxide has been replaced lately as a base with magnesium oxide (MgO) or magnesium hydroxide (Mg(OH)₂) for the oxygen delignification of sulphite pulps. However, because of the low alkalinity of MgO or Mg(OH)₂, the temperature of delignification with MgO or Mg(OH)₂ must be about 30°C higher than for the same process using NaOH as the delignification agent (see Luo et al., *supra*). Alternatively, the delignification rate can be increased in the O_{MgO} process by the addition of a very limited amount of NaOH, since small concentrations of sodium salts can be tolerated in the recovery system of magnesium-based sulphite process. However, the risk of contamination in the long run is such that this alternative does not represent a desirable selection.

Changing the alkali source in the oxygen delignification process from sodium hydroxide to magnesium oxide or magnesium hydroxide, as taught by Bokstrom et al. *supra,* decreases the selectivity of lignin to carbohydrate degradation. Moreover, the strength properties also decrease, as illustrated in the relationship between tear index versus tensile index of Fig. 6, by Luo et al. *supra*. For a given type of wood chips used as starting material, it is well known that sulphite pulps usually have strength properties inferior to that of kraft pulp, and a further decrease in strength properties during the delignification process is therefore unacceptable for commercial operations.

It is known that a post treatment stage with sodium borohydride on an oxidized pulp, such as ozone delignified pulp, leads to increased pulp viscosity. For example, it was reported by Chirat et aL in Holzforschung, 1994, 48 Suppl. 133, that a reduction treatment stage with 0.1% sodium borohydride increases the viscosity of ozone bleached pulp from DPᵥ of 710 to 920. The chemistry of sodium borohydride reduction is well understood: carbonyl groups present in carbohydrates are reduced to alcohol functionalities (B. Browning, Methods of Wood Chemistry, Vol. 2, P. 685, Interscience Publishers).

In addition, it is proposed by S. Beharic in Papir 20, December 1992, 3(4) pp. 11-15 to add sodium borohydride either before ozone bleaching or after peroxide bleaching to limit the reduction in pulp viscosity. Again, two stages are involved for this pulp treatment.

Accordingly, there is therefore a great need to develop an oxygen delignification process providing pulps with enhanced strength properties and increased viscosity. Preferably, a single stage bleaching process should be considered, wherein a reducing agent would be added *in situ*. This would represent a significant advance in pulp bleaching, and bring significant benefits to the industry, because the elimination of one treatment stage of pulp represents a significant capital cost reduction.

### SUMMARY OF THE INVENTION

In accordance with the present invention, there is now provided an improvement to oxygen delignification process of sulphite pulps. More specifically, the present invention comprises the conventional steps of oxygen delignification of sulphite pulp, namely treating a sulphite pulp slurry in a reactor under oxygen overpressure in the presence of an alkali source, over a period of time sufficient to complete delignification of the pulp, with the improvement comprising adding *in situ* an effective amount of a reducing agent substantially non-reactive with the oxygen, to provide delignified sulphite pulps with enhanced strength properties and increased viscosity.

The present oxygen delignification process is particularly advantageous for sulphite pulps when MgO or Mg(OH)₂ are used as the alkali source. Other possible alkali sources include Ca(OH)₂, NH₄OH, NaOH and the like. Reducing agents include sodium borohydride, sodium hydrosulphite and the like, with sodium borohydride being the most preferred.

In another aspect of the present invention, the process comprises a first stage wherein the sulphite pulp is treated with the reducing agent, and then washed and pressed if necessary, and a second conventional oxygen delignification stage. Although good results are obtained with the two-stage process, the single stage process is much preferred because of the elimination of washing and pressing operations required after treatment with the reducing agent in the two-stage process.

### IN THE DRAWINGS

Figure I illustrates the strength properties of O_{MgO + R}D_{O}Eₒₚ(DP) bleached pulp and those of O_{MgO}D_{O}Eₒₚ (DP) bleached pulp.

### DETAILED DESCRIPTION OF THE INVENTION

It is an object of the present invention to provide a single or two-stage oxygen delignification process of sulphite pulp which can minimize the carbohydrate degradation and thus enhance the strength properties of the sulphite pulp, as well as the viscosity. The present single stage process is most advantageous for MgO delignification of sulphite pulps.

It is also an object of the present invention to provide a two-stage oxygen delignification process of sulphite pulps which can minimize the carbohydrate degradation and thus enhance the strength properties of the sulphite pulp, as well as the viscosity. As for the single stage process, the two-stage process is also most advantageous for MgO delignification of sulphite pulps.

The present invention comprises the use of a small amount of a reducing agent, most preferably sodium borohydride, either before or during the oxygen delignification process. Preferred alkali source, as mentioned above, are MgO, Mg(OH)₂ and the like. The key feature of the unexpected results obtained with the present single stage process is that the activity of the reducing agent is substantially not affected by the overpressure of oxygen in the reaction media. The reducing agent and the alkali source may be added simultaneously, or the reducing agent is added to the pulp shortly before the alkali source. The reverse order of addition of reagents is also possible. Preferred experimental conditions for carrying the present single stage process are as follows: pH from 8 to 13; temperature of from 80 to 140°C; an oxygen overpressure of from [2,07 to 13,79]x10⁵ Pa (30 to 200 psi) a pulp consistency of from 1% to 50%; an addition of from 0.01% to 10% of sodium borohydride, an addition of MgO of from 0.2 to 10%; and a reaction time of from 0.1 to 4 hours. Most preferred conditions are: 127°C, 6,89x10⁵ Pa (100 psi) O₂ pressure; 10% pulp consistency; an addition of 0.1% of sodium borohydride, an addition of 2% MgO and a reaction time of 2 hours. It has been unexpectedly found that the addition of sodium borohydride in conventional magnesium oxide-based oxygen delignification process of sulphite pulp results in the production of pulps having an increased viscosity and improved strength properties when compared to pulp prepared in the same manner but without the addition of sodium borohydride.

In the case of a two-stage process, the experimental conditions for the oxygen delignification stage are the same as those above. With respect to the first stage, preferred conditions are as follows: 0.1% to 10% (by weight on pulp) of reducing agent is mixed with a pulp suspension at a pH of from 5 to 13 and maintained at a temperature of 20 to 100°C for a period of time of a few seconds up to 2 hours. The pulp is then washed conventionnally, for example with water, and pressed if necessary, to collect the pulp fibers which will be treated under the above oxygen delignification stage. It has been unexpectedly found that the treatment of sulphite pulp with sodium borohydride before treating the pulp with a conventional magnesium oxide-based oxygen delignification process results in the production of pulps having an increased viscosity and improved strength properties when compared to pulp prepared in the same manner but without the addition of sodium borohydride. Results hereinbelow will also show that if the pulp is first treated under oxygen delignification conditions and then with a reducing agent, the properties of the pulp are not as good as the single stage treated pulp, or two stage treated pulp wherein the treatment with reducing agent occurred before oxygen delignification.

The expression "enhanced strength properties" should be interpreted as meaning that the strength properties of the pulp are at least comparable, and generally better than those of pulp obtained from a bleaching sequence using chlorine or chlorine dioxide without oxygen delignification. Further, "increased viscosity" means that the viscosity is at least equivalent to that of eastern Canadian softwood sulphite pulp after conventional O_{MgO} delignification, i.e., typically about 25 mPa.s to about 45 mPa.s.

The following examples are provided for illustrating the present invention and should not be construed as limiting its scope.

### Example 1

40 g of eastern softwood sulphite pulp (kappa no. 26.0, pulp viscosity 40.1 mPa·s determined on the chlorite delignified pulp) in a pulp consistency of 28.5% is weighed into a beaker containing about 360 ml of water, resulting in a pulp consistency of about 10% and then disintegrated in a conventional manner, for example by a blender to be free from fiber bundles. 0.5 % sodium borohydride (by weight on pulp) is rapidly mixed with the pulp slurry prepared above (~ 400 ml). The slurry has a pulp consistency of 10% and contains about 2% MgO (by weight on pulp) and 0.2% MgSO₄ (by weight on pulp). The pulp slurry is subsequently transferred to a Parr pressure reactor preheated at a temperature of about 100°C. The O_{MgO+R} process, that is, conventional O_{MgO} technology with the addition of sodium borohydride *in situ*, is performed at about 127°C and 6,89x10⁵ Pa (100 psi) for 2 hours in a single stage. The resulting pulp with a kappa number of 14.0 is then bleached to full brightness (90% ISO) in accordance with the conventional D_{O}Eₒₚ (DP)
wherein
- Dₒ stands for a chlorine dioxide stage;
- Eₒₚ represents a peroxide reinforced oxidative stage; and
- (DP) means that no washing is performed between chlorine dioxide treatment and peroxide treatment sequence.

The detailed conditions of each stage in the D_{O}Eₒₚ(DP) sequence is provided in Table 1 below. The tear-tensile beating curve of the O_{MgO + R} D_{O}Eₒₚ (DP) bleached pulp is shown in Figure 1.

**Table 1**

| **Detailed Conditions of Each Stage in the D**_{**o**}**E**_{**op**}**(DP) Stage** | | | | |
|---|---|---|---|---|
| | **D**_{**o**} | **E**_{**op**} | **(DP)** | |
| | | | **D** | **P** |
| Consistency (%) | 3.5 | 10 | 11.5 | 10 |
| Time (min) | 12 | 30 | 145 | 70 |
| Temperature (°C) | 60 | 70 | 72 | 80 |
| O₂ pressure (psi) | - | 40 for 4 min. | - | - |
| Chemicals (% on pulp) | Kappa: 0.14 ClO₂:0.75 | H₂O₂: 0.8 NaOH:1.8 | ClO₂:0.4 | H₂O₂: 0.5 NaOH:0.7 |

### Example 2

This experiment is provided to illustrate the properties of a pulp obtained in experimental conditions similar to those of Example 1 without adding sodium borohydride during the conventional O_{MgO} process. As it will be seen, the strength properties of the O_{MgO} D_{O}Eₒₚ(DP) bleached pulp are inferior to those of the O_{MgO+R} D_{O}Eₒₚ(DP) bleached pulp.

The eastern softwood sulphite pulp (kappa no. 26.0, pulp viscosity 40.1 mPa.s determined on the chlorite delignified pulp) used in Example 1 is also used in the present example. 2 % MgO (by weight on pulp) and 0.2% MgSO₄ are mixed with a pulp suspension containing 40 g pulp. The pulp slurry is then transferred to a Parr pressure reactor preheated at a temperature of about 100°C. The O_{MgO} delignification process is performed at a temperature of 127°C with an oxygen overpressure of about 6,89x10⁵ Pa (100 psi) for 2 hrs. At the end of these 2 hours, the resulting pulp with a kappa number of 13.8 is then further bleached to a full brightness in accordance with the DₒEₒₚ(DP) sequence described above. The tear-tensile beating curve of the O_{MgO} Dₒ Eₒₚ (DP) bleached pulp is also illustrated in Figure 1, which shows that the strength properties of O_{MgO+R}D_{O}Eₒₚ(DP) bleached pulp are significantly improved over those of O_{MgO}D_{O}Eₒₚ (DP) bleached pulp.

### Example 3

This example is provided to show the effect of sodium borohydride concentration on the pulp viscosity after the O_{MgO+R} delignification process. An Eastern softwood sulphite pulp with a kappa no. of 25.2 and viscosity of 43.1 mPa·s determined on the chlorite delignified pulp is used. The sodium borohydride concentration varies from 0 to 0.05 to 0.1 to 0.2% (by weight on pulp). The required amount of NaBH₄ is rapidly mixed with a pulp slurry having a pulp consistency of 10% and containing about 2% MgO and about 0.2 % MgSO₄. The subsequent procedures are identical to those described in Example 1. The kappa number, viscosity and brightness of the O_{MgO+R} delignified pulps at various NaBH₄ concentrations are given in Table 2.

**Table 2**

| **Effect of the sodium borohydride concentration on pulp viscosity during the O**_{**MgO**} **process** | | | |
|---|---|---|---|
| Sodium borohydride concentration (% on pulp) | Kappa number | Pulp viscosity (mPa.s) | Brightness (% ISO) |
| 0 | 12.8 | 27.8 | 57.7 |
| 0.05 | 13.9 | 39.1 | 59.6 |
| 0.1 | 12.4 | 43.0 | 62.5 |
| 0.2 | 14.6 | 43.0 | 60.9 |

The above results clearly show that the pulp viscosity is significantly improved when sodium borohydride is present during the O_{MgO} delignification stage. In addition, the brightness of the O_{MgO+R} delignified is always higher than that of the O_{MgO} treated pulp under otherwise the same condition. Furthermore, the data show that a sodium borohydride concentration as low as 0.05% is sufficient to achieve the desired beneficial effect.

### Example 4

This example is provided to show that a two-stage RO_{MgO}, i.e., treatment with sodium borohydride in a first stage followed by water washing and then conventional O_{MgO} in a second stage, can produce acceptable delignified pulp with properties inferior to those of the O_{MgO+R} treated pulp.

The same Eastern softwood sulphite pulp as that used in Example 3 is used in this example. 0.1% NaBH₄ (by weight on pulp) is mixed with a pulp suspension of pH 9.5 and containing 20 g pulp in a polyethylene bag. Sodium hydroxide is used to increase the pH. The polyethylene bag is then thermostated at 50°C. At the completion of 30 minutes, the pulp slurry is thoroughly washed with purified water and the pulp fibres are collected for the subsequent O_{MgO} treatment under the conditions of 10% pulp consistency, 2% MgO, 0.2% MgSO₄, 6,89x10⁵ Pa (100 psi), 127°C, 2 h and without the addition of sodium borohydride. The kappa number, viscosity and pulp brightness of the resulting pulp are compared to those of O_{MgO} treated and O_{MgO+R} treated pulps in Table 3.

**Table 3**

| **Kappa number, viscosity and brightness obtained for pulp treated under different processes** | | | |
|---|---|---|---|
| **Technique** | **Kappa no.** | **Viscosity** (mPa.s) | **Brightness** (% ISO) |
| O_{MgO} | 12.8 | 27.8 | 57.7 |
| O_{MgO+R}(0.1% NaBH₄) | 12.4 | 43.0 | 62.5 |
| RO_{MgO} (0.1% NaBH₄) | 13.8 | 39.5 | 59.9 |

Table 3 shows that the results obtained for a pulp treated under the RO_{MgO} process are better than that treated under the O_{MgO} process. However, the best results are obtained with a single stage O_{MgO + R} process.

### Example 5

This example is provided to show that a reduction with sodium borohydride in a second stage after the O_{MgO} treatment of the pulp in a first stage, i.e., a O_{MgO}R sequence, also increases the pulp viscosity, but rather moderately. However, the viscosity of the O_{MgO}R treated pulp is substantially lower than that of the single stage O_{MgO+R} treated pulp according to the present invention.

The same Eastern softwood sulphite pulp as in Example 3 is used. 20 g of pulp is subjected to a first stage O_{MgO} process under the conditions of 10% pulp consistency, 2% MgO, 0.2% MgSO₄, 6,89 x 10⁵ Pa (100 psi), 127°C, 2h, without adding sodium borohydride. Subsequently, the O_{MgO} delignified pulp is treated in a second stage with 0.1% sodium borohydride at pH 9.5, 10% pulp consistency and 50°C for 30 minutes. The kappa number, the viscosity and the pulp brightness of the resulting pulp are compared to those of O_{MgO} treated and O_{MgO+R} treated pulps in Table 4.

**Table 4**

| **Kappa number, viscosity and brightness obtained for pulp treated under different processes** | | | |
|---|---|---|---|
| **Technique** | **Kappa no.** | **Viscosity** (mPa.s) | **Brightness** (% ISO) |
| O_{MgO} | 12.8 | 27.8 | 57.7 |
| O_{MgO+R}(0.1% NaBH₄) | 12.4 | 43.0 | 62.5 |
| O_{MgO}R(0.1% NaBH₄) | 12.0 | 32.9 | 63.3 |

The above results show that the viscosity of the O_{MgO}R treated pulp is about 5 units higher than that of the O_{MgO} treated pulp, however about 10 units lower than that of the O_{MgO+R} treated pulps.

In view of the above results, it is apparent that the addition of a reducing agent *in situ* during the oxygen delignification process provides pulps with a higher viscosity and increased strength properties than that obtained during two-stage processes wherein the reducing agent is added either prior to or after the oxygen delignification process. The combination of a two-stage operation into a single stage one is beneficial not only because one stage has been removed, but also because the physical properties of the resulting pulp are significantly better. Nevertheless, good results are also obtained with a two stage process wherein the treatment with the reducing agent is carried out before the oxygen delignification stage. For obvious reasons, as mentioned above, a single stage process is most preferred.

## Claims

1. A method for the oxygen delignification of sulphite pulp, the method comprising treating a sulphite pulp slurry in a reactor under oxygen overpressure at a pH of from 8 to 13 with an effective amount of an alkali source over a period of time sufficient to complete delignification of the sulphite pulp; and adding *in situ* an effective amount of a reducing agent substantially non-reactive with the oxygen to provide a sulphite pulp with enhanced strength properties and increased viscosity.

2. A method according to claim 1 wherein the alkali source comprises MgO, Mg(OH)₂, Ca(OH)₂, NH₄OH, NaOH or mixtures thereof, and the reducing agent comprises sodium borohydride or sodium hydrosulphite.

3. A method according to claim 1 wherein the alkali source and the reducing agent are added simultaneously in the reactor.

4. A method according to claim 1 wherein the reducing agent is added in the reactor before the alkali source.

5. A method according to claim 1 wherein the temperature of the reactor is maintained between 80 and 140°C with the oxygen overpressure being from [2,07 to 13,79]x10⁵ Pa (30 to 200 psi), a pulp consistency of from 1 to 50%, and the period of time is from 0.1 to 4 hours.

6. A method according to claim 1 wherein 0.01% to 10% of reducing agent is added, and 0.5 to 10% of alkali source is added.

7. A method for the oxygen delignification of sulphite pulp, the method comprising treating a pulp slurry in a reactor at a temperature of from 80 to 140°C under an oxygen overpressure and at a pH of from 9 to 12 with from 0.5 to 10% of an alkali source over a period of time sufficient to complete delignification of the pulp; and adding in the reactor simultaneously with the alkali source from 0.01 to 10% of a reducing agent substantially non-reactive with the oxygen, improve the strength properties and increased the viscosity of the pulp.

8. A method according to claim 7 wherein the alkali source comprises MgO and the reducing agent comprises sodium borohydride.

9. A method according to claim 7 wherein the oxygen overpressure is from [2,07 to 13,79]x10⁵Pa (30 to 200 psi) and the pulp consistency is from 1 to 50%.

10. A method for the oxygen delignification of sulphite pulp, the method comprising a first stage wherein a sulphite pulp suspension is treated with an effective amount of a reducing agent, and then washing and pressing the sulphite pulp in a conventional manner, and collecting the sulphite pulp; and a second stage wherein a sulphite pulp slurry is treated in a reactor under oxygen overpressure at a pH of from 8 to 13 with an effective amount of an alkali source over a period of time sufficient to complete delignification of the sulphite pulp, to provide a sulphite pulp with enhanced strength properties and increased viscosity.

11. A method according to claim 10 wherein the amount of reducing agent added in the first stage is from 0.01 to 10% (by weight on pulp) at a pH of from 5 to 13, and wherein the temperature in the first stage is maintained between 20 to 100°C for a period of time of a few seconds up to 2 hours.

12. A method according to claim 10 wherein the alkali source comprises MgO, Mg(OH)₂, Ca(OH)₂, NH₄OH, NaOH or mixtures thereof, and the reducing agent comprises sodium borohydride or sodium hydrosulphite.

13. A method according to claim 10 wherein the temperature of the reactor is maintained between 80 and 140°C with the oxygen overpressure being from [2,07 to 13,79]x10⁵ Pa (30 to 200 psi), a pulp consistency of from 1 to 50%.

14. A method for the oxygen delignification of sulphite pulp, the method comprising a first stage wherein a sulphite pulp suspension is treated with 0.01 to 10% of a reducing agent, and then washing and pressing the sulphite pulp in a conventional manner, and collecting the sulphite pulp; and a second stage wherein a sulphite pulp slurry is treated at a temperature of from 80 to 140°C in a reactor under oxygen overpressure at a pH of from 9 to 12 with 0.5 to 10% of an alkali source over a period of time sufficient to complete delignification of the sulphite pulp, to provide a sulphite pulp with enhanced strength properties and increased viscosity.

15. A method according to claim 14 wherein the alkali source comprises MgO and the reducing agent comprises sodium borohydride.

16. A method according to claim 14 wherein the oxygen overpressure is from [2,07 to 13,79]x10⁵ Pa (30 to 200 psi) and the pulp consistency is from 1 to 50%.

17. A method for the oxygen delignification of sulphite pulp comprising the steps of:
- treating a sulphite pulp slurry in a reactor under oxygen overpressure at a pH of from 8 to 13 with an effective amount of an alkali source over a period of time sufficient to complete delignification of the sulphite pulp wherein the alkali source is selected from the group consisting of MgO, Mg(OH)₂, Ca(OH)₂, NH₄OH, NaOH and mixtures thereof; and
- adding an effective amount of reducing agent which is substantially non-reactive with the oxygen to provide a sulphite pulp with enhanced strength properties and increased viscosity, with the proviso that reducing agent addition is carried out
i) in a separate stage before adding the alkali source in the reactor; or
ii) simultaneously with the alkali source in the reactor.

18. A method according to claim 17 wherein the temperature of the reactor is maintained between 80 and 140°C with the oxygen overpressure being from [2,07 to 13,79]x10⁵ Pa (30 to 200 psi) a pulp consistency of from 1 to 50%, and the period of time is from 0.1 to 4 hours.

19. A method according to claim 17 wherein 0.01% to 10% by weight pulp of reducing agent is added, and 0.5 to 10% by weight pulp, of alkali source is added.

20. A method according to claim 17 wherein the reducing agent comprises sodium borohydride or sodium hydrosulphite.

21. A method for the oxygen delignification of sulphite pulp comprising the steps of:
- treating a sulphite pulp slurry in a reactor at a temperature of from 80 to 140°C under oxygen overpressure at a pH of from 9 to 12 with from 0.5 to 10% by weight pulp of an alkali source over a period of time sufficient to complete delignification of the sulphite pulp, wherein the alkali source is selected from the group consisting of MgO, Mg(OH)₂, Ca(OH)₂, NH₄OH, NaOH and mixtures thereof; and
- adding in the reactor simultaneously with the alkali source from 0.01 to 10% by weight of pulp of sodium borohydride to improve strength properties and increase the viscosity of the sulphite pulp.

22. A method according to claim 21 wherein the oxygen overpressure is from [2,07 to 13,79) x 10⁵ Pa (30 to 200 psi) and the pulp consistency is from 1 to 50%.

23. A method for the oxygen delignification of sulphite pulp, the method comprising a first stage wherein a sulphite pulp suspension is treated with an effective amount of sodium borohydride, and then washing and pressing the sulphite pulp in a conventional manner, and collecting the sulphite pulp; and a second stage wherein a sulphite pulp slurry is in a reactor under oxygen overpressure at a pH of from 8 to 13 with an effective amount of an alkali source selected from the group consisting of MgO, Mg(OH)₂, Ca(OH)₂, NH₄OH, NaOH and mixtures thereof, over a period of time sufficient to complete delignification of the sulphite pulp, to provide a sulphite pulp with enhanced strength properties and increased viscosity.

24. A method according to claim 23 wherein the amount of sodium borohydride added in the first stage is from 0.01% to 10% by weight of pulp at a pH of from 8 to 13, and wherein temperature in the first stage is maintained between 20 and 100°C for a period of time of a few seconds up to 2 hours.

25. A method according to claim 19 wherein the oxygen overpressure is from [2,07 to 13,79]x10⁵ Pa (30 to 200 psi), and the pulp consistency is from 1 to 50%.

## Patentansprüche

1. Verfahren zur Sauerstoff-Delignifizierung von Sulfit-Pulpe, wobei das Verfahren die Behandlung einer Sulfit-Pulpenaufschlämmung in einem Reaktor unter Sauerstoff-Überdruck bei einem pH-Wert von zwischen 8 bis 13 mit einer wirksamen Menge einer Alkali-Quelle über einen Zeitraum, welcher zur vollständigen Delignifizierung der Sulfit-Pulpe ausreichend ist und die in-situ Zugabe einer wirksamen Menge eines im Wesentlichen mit dem Sauerstoff nicht reaktiven Reduktionsmittels umfasst, um eine Sulfit-Pulpe mit verbesserten Festigkeitseigenschaften und erhöhter Viskosität zu liefern.

2. Verfahren gemäß Anspruch 1, worin die Alkali-Quelle MgO, Mg(OH)₂, Ca(OH)₂, NH₄OH, NaOH oder Mischungen daraus umfasst und das Reduktionsmittel Natriumborhydrid oder Natriumhydrogensulfit umfasst.

3. Verfahren gemäß Anspruch 1, worin die Alkali-Quelle und das Reduktionsmittel gleichzeitig dem Reaktor zugesetzt werden.

4. Verfahren gemäß Anspruch 1, worin das Reduktionsmittel dem Reaktor vor der Alkali-Quelle zugesetzt wird.

5. Verfahren gemäß Anspruch 1, worin die Temperatur des Reaktors zwischen 80 und 140 °C gehalten wird, wobei der Sauerstoff-Überdruck [2,07 bis 13,79] x 10⁵ Pa (30 bis 200 psi), die Pulpenkonsistenz 1 bis 50% und die Zeitdauer von 0,1 bis 4 Stunden beträgt.

6. Verfahren gemäß Anspruch 1, worin 0,01% bis 10% Reduktionsmittel und 0,5 bis 10% Alkali-Quelle zugegeben werden.

7. Verfahren zur Sauerstoff-Delignifizierung von Sulfit-Pulpe, wobei das Verfahren die Behandlung einer Pulpenaufschlämmung in einem Reaktor bei einem Temperatur von 80 bis 140 °C unter einem Sauerstoff-Überdruck und bei einem pH-Wert von 9 bis 12 mit 0,5 bis 10% einer Alkali-Quelle über eine zur vollständigen Delignifizierung der Pulpe ausreichenden Zeitdauer und die gleichzeitig mit der Alkali-Quelle erfolgende Zugabe von 0,01 bis 10% eines im Wesentlichen mit dem Sauerstoff nicht reaktiven Reduktionsmittels umfasst, zur Verbesserung der Festigkeitseigenschaften und der Erhöhung der Viskosität der Pulpe.

8. Verfahren nach Anspruch 7, worin die Alkali-Quelle MgO und das Reduktionsmittel Natriumborhydrid umfasst.

9. Verfahren gemäß Anspruch 7, worin der Sauerstoff-Überdruck [2,07 bis 13,79] x 10⁵ Pa (30 bis 200 psi) und die Pulpenkonsistenz von 1 bis 50% beträgt.

10. Verfahren zur Sauerstoff-Delignifizierung von Sulfit-Pulpe, wobei das Verfahren eine erste Stufe, worin eine Sulfit-Pulpensuspension mit einer wirksamen Menge eines Reduktionsmittels behandelt wird und dann die Sulfit-Pulpe in herkömmlicher Weise gewaschen und verpresst und die Sulfit-Pulpe gesammelt wird und eine zweite Stufe umfasst, worin eine Sulfit-Pulpenaufschlämmung in einem Reaktor unter Sauerstoff-Überdruck bei einem pH-Wert von 8 bis 13 mit einer wirksamen Menge einer Alkali-Quelle über eine Zeitdauer behandelt wird, welche ausreicht, um die Delignifizierung der Sulfit-Pulpe zu vervollständigen, um eine Sulfit-Pulpe mit verbesserten Festigkeitseigenschaften und erhöhter Viskosität zu liefern.

11. Verfahren gemäß Anspruch 10, worin die Menge an in der ersten Stufe zugegebenem Reduktionsmittel 0,01 bis 10% (pro Gewicht an Pulpe) bei einem pH-Wert von 5 bis 13 beträgt und worin die Temperatur während der ersten Stufe zwischen 20 bis 100 °C für eine Zeitdauer von wenigen Sekunden bis zu 2 Stunden gehalten wird.

12. Verfahren gemäß Anspruch 10, worin die Alkali-Quelle MgO, Mg(OH)₂, Ca(OH)₂, NH₄OH, NaOH oder Mischungen daraus umfasst und das Reduktionsmittel Natriumborhydrid oder Natriumhydrogensulfit umfasst.

13. Verfahren gemäß Anspruch 10, worin die Temperatur des Reaktors zwischen 80 und 140 °C gehalten wird, wobei der Sauerstoff-Überdruck [2,07 bis 13,79] x 10⁵ Pa (30 bis 200 psi) und die Pulpenkonsistenz von 1 bis 50% beträgt.

14. Verfahren zur Sauerstoff-Delignifizierung von Sulfit-Pulpe, wobei das Verfahren eine erste Stufe, worin eine Sulfit-Pulpensuspension mit 0,01 bis 10% eines Reduktionsmittels behandelt wird, dann die Sulfit-Pulpe in einer herkömmlichen Weise gewaschen und verpresst und die Sulfit-Pulpe gesammelt wird, und eine zweite Stufe umfasst, worin eine Sulfit-Pulpenaufschlämmung bei einer Temperatur von 80 bis 140 °C in einem Reaktor unter Sauerstoff-Überdruck bei einem pH-Wert von 9 bis 12 mit 0,5 bis 10 % einer Alkali-Quelle über eine zur Vervollständigung der Delignifizierung der Sulfit-Pulpe ausreichenden Zeit behandelt wird, um eine Sulfit-Pulpe mit verbesserter Festigkeit und erhöhter Viskosität zu erhalten.

15. Verfahren gemäß Anspruch 14, worin die Alkali-Quelle MgO und das Reduktionsmittel Natriumborhydrid umfasst.

16. Verfahren gemäß Anspruch 14, worin der Sauerstoff-Überdruck [2,07 bis 13,79] x 10⁵ Pa (30 bis 200 psi) und die Pulpenkonsistenz von 1 bis 50% beträgt.

17. Verfahren zur Sauerstoff-Delignifizierung von Sulfit-Pulpe umfassend die Stufen:
- Behandlung einer Sulfit-Pulpenaufschlämmung in einem Reaktor unter Sauerstoff-Überdruck bei einem pH-Wert von 8 bis 13 mit einer wirksamen Menge einer Alkali-Quelle über eine zur vollständigen Delignifizierung der Sulfit-Pulpe ausreichenden Zeitdauer, worin die Alkali-Quelle aus der Gruppe ausgewählt wird, die aus MgO, Mg(OH)₂, Ca(OH)₂, NH₄OH, NaOH und Mischungen daraus besteht und
- die Zugabe einer wirksamen Menge eines Reduktionsmittels, das im Wesentlichen nicht-reaktiv mit dem Sauerstoff ist, um eine Sulfit-Pulpe mit verbesserten Festigkeitseigenschaften und erhöhter Viskosität zu liefern, mit der Maßgabe, dass die Reduktionsmittelzugabe
- i) einer getrennten Stufe vor dem Zusetzen der Alkali-Quelle in den Reaktor oder
- ii) gleichzeitig mit der Alkali-Quelle erfolgt.

18. Verfahren gemäß Anspruch 17, worin die Temperatur des Reaktors zwischen 80 und 140 °C gehalten wird, wobei der Sauerstoff-Überdruck [2,07 bis 13,79] x 10⁵ Pa (30 bis 200 psi), die Pulpenkonsistenz 1 bis 50% und die Zeitdauer 0,1 bis 4 Stunden beträgt.

19. Verfahren gemäß Anspruch 17, worin 0,01 bis 10 Gew% (bezogen auf das Gewicht der Pulpe) an Reduktionsmittel und 0,5 bis 10 Gew% (bezogen auf das Gewicht der Pulpe) der Alkali-Quelle zugegeben werden.

20. Verfahren gemäß Anspruch 17, worin das Reduktionsmittel Natriumborhydrid oder Natriumhydrogensulfit umfasst.

21. Verfahren zur Sauerstoff-Delignifizierung von Sulfit-Pulpe, umfassend die Stufen:
- die Behandlung einer Sulfit-Pulpenaufschlämmung in einem Reaktor bei einem Temperatur von 80 bis 140 °C unter einem Sauerstoff-Überdruck bei einem pH-Wert von 9 bis 12 mit von 0,5 bis 10 Gew% (bezogen auf das Gewicht Pulpe) einer Alkali-Quelle über eine zur Vervollständigung der Delignifizierung der Sulfit-Pulpe ausreichenden Zeitdauer, worin die Alkali-Quelle aus der Gruppe ausgewählt wird, die aus MgO, Mg(OH)₂, Ca(OH)₂, NH₄OH, NaOH und Mischungen daraus besteht und,
- die gleichzeitig mit der Alkali-Quelle erfolgende Zugabe von 0,01 bis 10 Gew% (bezogen auf das Gewicht Pulpe) Natriumbohrhydrid, zur Verbesserung der Festigkeitseigenschaften und Erhöhung der Viskosität der Sulfit-Pulpe.

22. Verfahren gemäß Anspruch 21, worin der Sauerstoff-Überdruck [2,07 bis 13,79] x 10⁵ Pa (30 bis 200 psi) und die Pulpenkonsistenz 1 bis 50% beträgt.

23. Verfahren zur Sauerstoff-Delignifizierung von Sulfit-Pulpe, wobei das Verfahren eine erste Stufe, worin eine Sulfit-Pulpensuspension mit einer wirksamen Menge Natriumborhydrid behandelt wird und dann die Sulfit-Pulpe in einer herkömmlichen Weise gewaschen und verpresst und die Sulfit-Pulpe gesammelt wird und eine zweite Stufe umfasst, worin eine Sulfit-Pulpenaufschlämmung sich in einem Reaktor unter Sauerstoff-Überdruck bei einem pH-Wert von 8 bis 13 mit einer wirksamen Menge einer Alkali-Quelle vorliegt, welche aus der Gruppe ausgewählt wird, die aus MgO, Mg(OH)₂, Ca(OH)₂, NH₄OH, NaOH und Mischungen daraus besteht, über eine zur Vervollständigung der Delignifizierung der Sulfit-Pulpe ausreichende Zeitdauer, um eine Sulfit-Pulpe mit verbesserten Festigkeitseigenschaften und erhöhter Viskosität zu liefern.

24. Verfahren gemäß Anspruch 23, worin die Menge an Natriumborhydrid, die in der ersten Stufe zugegeben wird 0,01 % bis 10 Gew% (pro Gewicht Pulpe) bei einem pH-Wert von 8 bis 13 beträgt und worin die Temperatur in der ersten Stufe zwischen 20 und 100 °C für eine Zeitdauer von wenigen Sekunden bis zu 2 Stunden gehalten wird.

25. Verfahren gemäß Anspruch 19, worin der Sauerstoff-Überdruck [2,07 bis 13,79] x 10⁵ Pa (30 bis 200 psi) und die Pulpenkonsistenz 1 bis 50% beträgt.

## Revendications

1. Procédé de délignification par oxygène d'une pâte au bisulfite, ledit procédé comprenant le traitement d'une pâte au bisulfite dans un réacteur en surpression d'oxygène, à un pH de 8 à 13, en présence d'un quantité suffisante d'un alcali actif, pendant un laps de temps suffisant pour compléter la délignification de ladite pâte au bisulfite; et l'ajout *in situ* d'un quantité suffisante d'un agent réducteur en grande partie non réactif à l'oxygène afin d'obtenir une pâte au bisulfite ayant des propriétés améliorées au niveau de la résistance et disposant d'une plus grande viscosité.

2. Procédé selon la revendication 1, dans lequel l'alcali actif est choisi parmis MgO, Mg(OH)₂, Ca(OH)₂, NH₄OH, NaOH ou des mélanges de ceux-ci et l'agent réducteur est choisi parmi le borohydrure de sodium et l'hydrosulfite de sodium.

3. Procédé selon la revendication 1, dans lequel l'alcali actif et l'agent réducteur sont ajoutés simultanément au réacteur.

4. Procédé selon la revendication1, dans lequel l'agent réducteur est ajouté au réacteur avant l'alcali actif.

5. Procédé selon la revendication 1, dans lequel la température du réacteur est maintenue entre 80 et 140°C, dans une surpression en oxygène de 2,07 à 13,79 X 10⁵ Pa, à une consistance de 1 à 50% pour un laps de temps de 0.1 à 4 heures.

6. Procédé selon la revendication 1, dans lequel 0.01% à 10% d'agent réducteur et 0.5 à 10% d'alcali actif sont ajoutés au réacteur.

7. Procédé de délignification par oxygène d'une pâte au bisulfite, ledit procédé comprenant le traitement d'une pâte au bisulfite dans un réacteur maintenu à une température entre 80 et 140°C, en surpression en oxygène, à un pH de 9 à 12 en présence de 0.5 à 10% d'un alcali actif pendant un laps de temps suffisant pour compléter la délignification de ladite pâte au bisulfite; et l'ajout au réacteur, simultanément à l'ajout de l'alcali actif de 0.01 à 10% d'un agent réducteur en grande partie non réactif à l'oxygène afin d'obtenir une pâte au bisulfite ayant des propriétés améliorées au niveau de la résistance et disposant d'une plus grande viscosité.

8. Procédé selon la revendication 7, dans lequel l'alcali actif comprend le MgO et l'agent réducteur comprend le borohydrure de sodium.

9. Procédé selon la revendication 7, dans lequel la surpression en oxygène est de 2,07 à 13,79 X 10⁵ Pa et la consistance est de 1 à 50%.

10. Procédé de délignification par oxygène d'une pâte au bisulfite, ledit procédé comprenant une première étape dans laquelle la pâte au bisulfite est traitée à l'aide d'une quantité suffisante d'agent réducteur, suivi d'un lavage et pressage conventionel de la pâte au bisulfite, suivi d'une récupération de la pâte au bisulfite ainsi traitée; et une seconde étape dans laquelle la pâte traitée et receuillie dans la première étape subie un traitement dans un réacteur en surpression d'oxygène à un pH de 8 à 13 en présence d'un quantité suffisante d'un alcali actif pendant un laps de temps suffisant pour compléter la délignification de ladite pâte au bisulfite afin d'obtenir une pâte au bisulfite ayant des propriétés améliorées au niveau de la résistance et disposant d'une plus grande viscosité.

11. Procédé selon la revendication 10, dans lequel la quantité d'agent réducteur ajoutée lors de la première étape est de 0.01 à 10% (basé sur le poids de la pâte au bisulfite), à un pH de 5 à 13, à une température de première étape maintenue entre 20 et 100°C pour un laps de temps variant de quelques secondes à 2 heures.

12. Procédé selon la revendication 10, dans lequel l'alcali actif est choisi parmis MgO, Mg(OH)₂, Ca(OH)₂, NH₄OH, NaOH ou des mélanges de ceux-ci et l'agent réducteur est choisi parmi le borohydrure de sodium et l'hydrosulfite de sodium.

13. Procédé selon la revendication 10, dans lequel la température du réacteur est maintenue entre 80 et 140°C, dans une surpression en oxygène de 2,07 à 13,79 X 10⁵ Pa, à une consistance de 1 à 50%.

14. Procédé de délignification par oxygène d'une pâte au bisulfite, ledit procédé comprenant une première étape dans laquelle la pâte au bisulfite est traitée à l'aide de 0.01 à 10% d'agent réducteur, suivi d'un lavage et pressage conventionel de la pâte au bisulfite, suivi d'une récupération de la pâte au bisulfite ainsi traitée; et une seconde étape dans laquelle la pâte traitée et recueillie dans la première étape subie un traitement dans un réacteur en surpression d'oxygène, à une température de 80 à 140°C, à un pH de 9 à 12 en présence de 0.5 à 10% d'un alcali actif pendant un laps de temps suffisant pour compléter la délignification de ladite pâte au bisulfite afin d'obtenir une pâte au bisulfite ayant des propriétés améliorées au niveau de la résistance et disposant d'une plus grande viscosité.

15. Procédé selon la revendication 14, dans lequel l'alcali actif comprend le MgO et l'agent réducteur comprend le borohydrure de sodium.

16. Procédé selon la revendication 14, dans lequel la surpression en oxygène est de 2,07 à 13,79 X 10⁵ Pa et la consistance est de 1 à 50%.

17. Procédé de délignification par oxygène d'une pâte au bisulfite, ledit procédé comprenant les étapes suivantes :
- traitement de la pâte au bisulfite dans un réacteur en surpression d'oxygène à un pH de 8 à 13 en présence d'une quantité suffisante d'un alcali actif pendant un laps de temps suffisant pour compléter la délignification de ladite pâte au bisulfite, dans lequel traitement la source d'alcali actif est choisie parmis l'ensemble de MgO, Mg(OH)₂, Ca(OH)₂, NH₄OH, NaOH et des mélanges de ceux-ci; et
- ajout d'un agent réducteur en grande partie non réactif à l'oxygène afin d'obtenir une pâte au bisulfite ayant des propriétés améliorées au niveau de la résistance et disposant d'une plus grande viscosité, à la condition que l'ajout de l'agent réducteur se fasse :
i) lors d'une étape préalable à l'ajout de l'alcali actif au réacteur; ou
ii) simultanément à l'ajout de l'alcali actif au réacteur.

18. Procédé selon la revendication 17, dans lequel la température du réacteur est maintenue entre 80 et 140°C, dans une surpression en oxygène de 2,07 à 13,79 X 10⁵ Pa, à une consistance de 1 à 50% pour un laps de temps de 0.1 à 4 heures.

19. Procédé selon la revendication 17, dans lequel 0.01% à 10% d'agent réducteur et 0.5 à 10% d'alcali actif sont ajoutés au réacteur.

20. Procédé selon la revendication 17, dans lequel l'agent réducteur est choisi parmi le borohydrure de sodium et l'hydrosulfite de sodium.

21. Procédé de délignification par oxygène d'une pâte au bisulfite, ledit procédé comprenant les étapes suivantes :
- traitement de la pâte au bisulfite dans un réacteur en surpression d'oxygène à une température entre 80 et 140°C, à un pH de 9 à 12 en présence de 0.5 à 10% basé sur le poids de ladite pâte d'un alcali actif pendant un laps de temps suffisant pour compléter la délignification de ladite pâte au bisulfite, dans lequel traitement la source d'alcali actif est choisie parmis l'ensemble de MgO, Mg(OH)₂, Ca(OH)₂, NH₄OH, NaOH et des mélanges de ceux-ci; et
- ajout, simultané à l'ajout de l'alcali actif, de 0.01 à 10%, basé sur le poids de ladite pâte, d'un agent réducteur en grande partie non réactif à l'oxygène afin d'obtenir une pâte au bisulfite ayant des propriétés améliorées au niveau de la résistance et disposant d'une plus grande viscosité.

22. Procédé selon la revendication 21, dans lequel la surpression en oxygène est de 2,07 à 13,79 X 105 Pa et la consistance est de 1 à 50%.

23. Procédé de délignification par oxygène d'une pâte au bisulfite, ledit procédé comprenant une première étape dans laquelle une suspension de la pâte au bisulfite est traitée à l'aide d'une quantité suffisante d'hybrohydrure de sodium, suivi d'un lavage et pressage conventionel de la pâte au bisulfite, suivi d'une récupération de la pâte au bisulfite ainsi traitée; et une seconde étape dans laquelle la pâte traitée et recueillie dans la première étape subie un traitement dans un réacteur en surpression d'oxygène, à un pH de 8 à 13, en présence d'une quantité suffisante d'une source d'alcali actif choisie parmis l'ensemble de MgO, Mg(OH)₂, Ca(OH)₂, NH₄OH, NaOH et des mélanges de ceux-ci; et pendant un laps de temps suffisant pour compléter la délignification de ladite pâte au bisulfite afin d'obtenir une pâte au bisulfite ayant des propriétés améliorées au niveau de la résistance et disposant d'une plus grande viscosité.

24. Procédé selon la revendication 23, dans lequel la quantité d'hybrohydrure de sodium ajoutée lors de la première étape est de 0.01 à 10%, basé sur le poids de la pâte, à un pH de 8 à 13, la température lors de la première étape étant maintenue entre 20 et 100°C pour un laps de temps de quelques secondes à 2 heures.

25. Procédé selon la revendication 19, dans lequel la surpression en oxygène est de 2,07 à 13,79 X 10⁵ Pa et la consistance est de 1 à 50%.
